

1

3,033,788

## FOAM INHIBITED LUBRICATING OIL COMPOSITION

Charles E. Trautman, Cheswick, Pa., assignor to Gulf Research & Development Company, Pittsburgh, Pa., a corporation of Delaware  
No Drawing. Filed Mar. 19, 1958, Ser. No. 722,391  
21 Claims. (Cl. 252—49.6)

This invention relates to the prevention of foaming of hydrocarbon oils, particularly mineral oils and lubricants containing them.

Hydrocarbon oils and oil compositions containing them tend to foam or froth when agitated in the presence of gases or vapors, such as air, steam, oil vapor, products of combustion, and the like. The amount of foam or froth varies with the conditions under which the oil compositions are agitated, as well as the characteristics of the composition. Under some conditions, the volume of foam or froth produced is many times that of the original oil, and even with mild agitation, substantial amounts of foam are produced in many oil compositions. In preparing and using such oils and oil compositions commercially, they are subjected to agitation under a wide range of conditions and frequently undesirable amounts of foam or froth are produced.

Various means of combating such foaming of oils and oil compositions have been proposed. For instance, mechanical devices have been proposed for destroying or breaking foam as it is formed. Usually such devices have been cumbersome or inefficient, or both, and they are not generally used commercially. Likewise, the incorporation of certain oil-soluble compounds in the oil has been proposed as a means for preventing foaming, such compounds being called "anti-foam agents." Unfortunately, no agent of this type has been found which is completely satisfactory in all types of oils under all conditions of use. While some agents have effectively reduced foaming of oils maintained at room temperature, i.e., about 70° to about 80° F., the agents have been less effective in oils maintained at an elevated temperature. Some agents have effectively reduced foaming in light oils but they have been less effective in heavier oils, i.e., oils having a viscosity above about 100 SUS at 100° F. Some of the prior so called "anti-foam agents" have been found even to increase the amount of foam formed in mineral oils maintained at about 200° F., particularly in the heavier oils, i.e., oils having a viscosity above about 100 SUS at 100° F.

It is important to provide an oil which is markedly resistant to foaming at an elevated temperature as well as at room temperature. For example, in the lubrication of internal combustion engines such as automotive, aviation, diesel and like engines, the temperature of the oil in the crankcase during engine operation is usually within the range of about 100° to about 225° F. In lubricating such engines, appreciable foaming of the oil seriously interferes with effective lubrication. By the present invention such foaming is effectively reduced. My new anti-foam agents and compositions are also useful in other hydrocarbon oils and oil compositions in which they are substantially insoluble whether used as a lubricant or not and whether the temperature of the oil is at room temperature or at an elevated temperature. The anti-foam agents and compositions of the present invention, however, are particularly effective in combating foaming in mineral oils, especially the heavier mineral oils and lubricants at temperatures between about 100° and 225° F.

It is therefore among the objects achieved by this invention to provide an improved method of preventing

2

foaming of hydrocarbon oils, particularly mineral oils and oil compositions containing them, in which the normal foaming tendency of the oil is effectively abated or suppressed for long periods of use without deleteriously affecting the other properties of the oil.

Another object achieved by the present invention is the provision of new and improved anti-foam agents and compositions capable of abating and inhibiting foaming of hydrocarbon oils and oil compositions when dispersed

10 therein in minute amounts.

A further object achieved by the present invention is the provision of new and improved oil compositions, particularly improved mineral oils and lubricants having marked resistance to foaming and other advantageous properties including resistance to emulsification and containing minute amounts of an oil-insoluble anti-foam agent finely dispersed therein.

I have discovered that the foaming of hydrocarbon oils, particularly mineral oils and compositions containing them, can be effectively suppressed or prevented without substantial modification of the desirable properties of such oils by forming in the oil a stable, fine dispersion of a small amount of an organo-silicate which has been subjected to ionizing radiation for a time sufficient for said organo-silicate to absorb at least about 6 megareps. of radiation. I have found that an oil containing such an irradiated organo-silicate as a stable, finely dispersed phase is markedly resistant to foaming even under the most violent conditions encountered in commercial practice. The presence of the finely dispersed irradiated organo-silicate in the oil apparently causes the film of the oil foam to rupture thereby quickly destroying the foam. In fact, particularly when an adequate amount of irradiated organo-silicate is used, its presence so rapidly breaks the oil foam that substantially all foam is destroyed as fast as it is formed.

I have found that an anti-foam agent comprising an organo-silicate can be converted to an improved product by subjecting the organo-silicate to ionizing radiation for a time sufficient for said organo-silicate to absorb at least about 6 megareps. of radiation while removing heat therefrom at a rate sufficient to maintain the bulb temperature of the organo-silicate below its decomposition or vaporization point. For example, I have found that in order to obtain a product which will materially reduce the foaming of an oil having a viscosity above about 100 SUS at 100° F. at temperatures up to about 225° F., the total amount of energy absorbed by the organo-silicate should be at least about 6, preferably between 50 about 6 and about 1000 megareps. If less than 6 megareps. of energy is absorbed, the irradiated product is not substantially improved with respect to its anti-foam properties for heavy oils over the unirradiated organo-silicate. While more than about 1000 megareps. of energy can be absorbed by the organo-silicate, the increment of improvement per megarep. of energy absorbed may be progressively smaller, thus rendering further irradiation economically unattractive. A megarep. (mrep.) is equal to one million reps. A rep. is defined as that dose of 60 any ionizing radiation which produces energy absorption of 83.8 ergs per gram of material.

While the total amount of energy which must be absorbed by the organo-silicate to obtain the desired product is critical, extreme care must be exercised in irradiating the organo-silicate. During irradiation the organo-silicate absorbs the high energy particles which are moving at a high rate of speed. This movement is transferred upon absorption in part into heat. If irradiation is left uncontrolled and is permitted to proceed at too great a rate, the temperature of the organo-silicate being treated can be raised to such a level that appreciable decomposition and degradation thereof takes place. Desirably the

organo-silicate being irradiated should be maintained during the irradiation period at a temperature as near the organo-silicate input temperature as possible so that the changes taking place in the organo-silicate are those resulting from irradiation rather than from heat.

Heat resulting from irradiation can be removed from the organo-silicate in many ways. One method comprises subjecting the organo-silicate to ionizing radiation, removing the organo-silicate from the radiation zone as the temperature thereof rises, reducing the temperature of the organo-silicate to a low temperature, such as about 70° to about 150° F., by recycling to a cooling zone, recycling said cooled organo-silicate to the radiation zone, and thereafter continuing such cycle until the organo-silicate has absorbed the required amount of energy. Another method, though not preferred, because of the poor heat conductivity of an organo-silicate, resides in the use of cooling coils immersed in the organo-silicate being irradiated to remove the heat therefrom.

The time required for irradiation is extremely important from an economic point of view. When the process is carried out over an extended period of time, it becomes unattractive for commercial use. At the same time, irradiating the organo-silicate in too short a time makes it extremely difficult to control the reaction and to maintain the organo-silicate within the desired temperature limits. I have found, for example, that an irradiation period per gram of material being irradiated of about 0.1 to about 20 seconds is sufficient to effect the desired result if a 2 million volt Van de Graaff accelerator producing an electron beam at an output of 500 watts is used. With other power sources, of course, the time will be changed in accordance with the power of the source. Provided heat is removed at a rate sufficient to prevent substantial decomposition or vaporization of the organo-silicate, any irradiation rate can be employed, though extremely high rates may involve technical difficulties.

I do not wish to limit this invention to any particular method of radiation inasmuch as the effects of radiation on organo-silicates are essentially the same insofar as anti-foam characteristics are concerned regardless of the radiation source. Ionizing radiations can be obtained, for example, using radio isotopes, nuclear reactors or high energy particle accelerators. Examples of radio isotopes which can be used are cobalt 60 for gamma and strontium 90 for beta. Operating nuclear reactors of intermediate or full power size can be used as a source for either gamma rays or neutrons or both. Particle accelerators such as the cyclotron, bevatron, synchrotron, Van de Graaff, or X-ray machines can also be used.

In effecting irradiation of the organo-silicate, the organo-silicate can be introduced into a well in a nuclear reactor or through a tube which traverses the reactor. In some instances where it is desirable to expose the organo-silicate to fast or high energy neutrons only, and in the substantial absence of beta and gamma radiation, the irradiation can be conducted outside of the reactor using a collimated beam of fast neutrons. Such a collimated beam of fast neutrons can be obtained, for example, as described in U.S. Patent No. 2,708,656 to Enrico Fermi and Leo Szilard, by inserting a hollow shaft or tube into the central portion of the reactor. Gamma rays can be screened from the fast neutron beam by means of a sheet of bismuth metal extending across the path of the beam.

A neutron-free radiation source can be obtained directly from a homogeneous reactor by separating the radioactive fission gases, xenon and krypton, from the reactor core by conventional or modified gas-liquid separating means. A continuous supply of the radioactive fission gases could be obtained from such a reactor. The fission gases have a very high intensity of beta and gamma radiation but a very short half life. These gases possess about one percent of the total fission energy. The gases are chemically

inert and therefore would not form undesired side reaction products.

While I am not certain as to the exact nature of the changes which take place when an organo-silicate is subjected to ionizing radiation, it is possible that some cross linking occurs. However, I have noted no significant change in viscosity of a tetra alkyl ortho silicate when irradiated to dosages of 6 to 50 megareps. of radiation. The viscosity and acid values of unirradiated and irradiated tetra(diisobutyl carbonyl)silicate for example, are as follows:

## VISCOSEITY

| 15      | Dosage Mreps. | 100° F. |      | 210° F. |      | Neut. Value<br>ASTM<br>(D-974) |
|---------|---------------|---------|------|---------|------|--------------------------------|
|         |               | CS      | SUS  | CS      | SUS  |                                |
| 20      | 0.....        | 15.15   | 78.0 | 3.39    | 37.5 | 63                             |
| 6.....  | 14.44         | 75.3    | 3.30 | 37.3    | 63   |                                |
| 24..... | 13.51         | 71.7    | 3.17 | 36.8    | 62   |                                |
| 50..... | 14.20         | 74.3    | 3.28 | 37.2    | 62   |                                |

It will be noted that the viscosity and acid values of tetra(diisobutyl carbonyl)silicate were not significantly changed by irradiation.

In the practice of this invention, various irradiated oil-insoluble liquid organo-silicates having a surface tension lower than that of the oil and capable of being stably and finely dispersed in the oil may be employed as anti-foam agents.

The organo-silicates which are irradiated for use according to this invention are composed of one or more silicon atoms, each silicon atom having attached to it at least one (OR) radical.

When more than one silicon atom is present, the silicon atoms are linked together through an oxygen atom. Typical organo-silicates which are suitable for the purpose of the invention are the irradiated liquid alkyl ortho silicates, aryl ortho silicates, aralkyl ortho silicates, aralkyl ortho silicates, alkaryl ortho silicates and heterocyclic ortho silicates, including their irradiated condensation or polymerization products.

The organo-silicates when polymerized may be straight chain products or they may be products of cross polymerization or a mixture of straight chain and cross linked polymers. Thus, the organo-silicates useful for the purpose of my invention may be represented by the formulae



60 65 in which the several R's represent the same or different alkyl, aryl, aralkyl, alkaryl or heterocyclic group and n is a number from 0 to 100 or higher depending upon the number of organo-silicate residues in the complex molecule. It will be understood that the formula showing cross polymerization is merely illustrative of cross polymerization products suitable for the purpose of my invention and such products may take other forms in which two or more cross linkings between polymers are estab-

lished. Such compounds may take a form in which they resemble cyclic compounds for example:



in which the several R's may be similar or dissimilar alkyl, aryl, aralkyl, alkaryl or heterocyclic groups.

The molecular weight and other properties of the organo-silicate vary with the particular organic radicals present and with the extent of polymerization where polymers are utilized. While some of them are resinous or rubbery solids, others are oily liquids. For the purpose of the present invention, the compounds which are liquid under normal conditions of temperature and pressure are contemplated.

The organo-silicates represented by Formulae I and II above wherein R is an alkyl group form a preferred class of compounds in that these compounds are generally more receptive to ionizing radiation than the compounds containing aryl or heterocyclic groups. Of the alkyl substituted compounds, it is preferred to employ those wherein the alkyl radical contains from 1 to 16 carbon atoms and n is a number from 0 to 100. While compounds containing higher alkyl groups can be utilized, if they are liquids insoluble in mineral oils, such compounds may be less effective. Regardless of whether the organo-silicate is a monomer, dimer, trimer or higher polymerized product, the organo-silicate preferably contains a minimum total of 10 carbon atoms. Thus, in Formula I above when R is a methyl radical, n is preferably at least 3. When R in Formula I is an ethyl radical, n is preferably at least 1. When R in Formula I is a propyl radical, n is zero or more. In Formula II, when R is a methyl radical, n is zero or more. Generally preferred for the present purpose are the relatively high molecular weight irradiated monomers where n is zero and R is an alkyl group containing from 8 to 16 carbon atoms. Thus, a preferred class of compounds include tetra octyl ortho silicate, tetra nonyl ortho silicate, tetra decyl ortho silicate, tetra undecyl ortho silicate, tetra dodecyl ortho silicate, tetra tridecyl ortho silicate, tetra tetradecyl ortho silicate, tetra pentadecyl ortho silicate, and tetra hexadecyl ortho silicate.

The lower molecular weight compounds, such as when R is a methyl or ethyl radical, are polymerized relatively easily and n in such a case may range from 3 to 100 or more. The higher molecular weight compounds, such as when R is a cetyl radical, are more difficult to condense or polymerize so that the resulting condensation or polymerization product may be only a dimer or trimer. Whether the silicate is only a monomer or a highly polymerized product, I prefer to employ an irradiated organo-silicate containing a minimum total of 10 carbon atoms. Particularly good anti-foam characteristics are obtained with an irradiated organo-silicate containing a minimum total of 32 to 40 carbon atoms and especially tetra(diisobutyl carbonyl) silicate which contains a total of 36 carbon atoms.

Many of the organo-silicates utilized according to the present invention are available commercially and therefore their preparation constitutes no part of the invention. Thus, commercially available organo-silicates are

obtained and then subjected to ionizing radiation for a time sufficient for them to absorb at least about 6 megareps. of radiation. The irradiated organo-silicates are then dispersed in the oil.

In the preparation of the lower molecular weight monomers, such as tetra methyl ortho silicate and tetra ethyl ortho silicate, one mol of a silicon halide such as silicon tetrachloride is reacted with four mols of the corresponding alcohol. To obtain the corresponding condensation products the tetra alkyl ortho silicates are further heated at refluxing temperature in the presence of water. In the course of preparing the monomers, four mols of hydrogen chloride are produced for every mol of tetra alkyl ortho silicate. The hydrogen chloride thus formed usually converts some of the alcohol to the ether or alkyl halide and produces water. The water thus formed may give rise to the condensation of the intermediate alkoxychlorosilane to form condensed esters such as hexaalkoxydisiloxane, octaalkoxytrisiloxane, decaalkoxytetrasiloxane, and the like.

The higher molecular weight ortho silicates can be obtained by an ester exchange reaction with a lower molecular weight ortho silicate. Tetra octyl ortho silicate can, for example, be prepared by an ester exchange reaction with tetra methyl ortho silicate or tetra ethyl ortho silicate. The ester exchange reaction can be effected, for example, by heating tetra ethyl ortho silicate with the desired alcohol or mercaptan in the presence of a catalyst such as benzene sulfonic acid or sodium ethoxide. The ester exchange reaction is conducted at a temperature of about 100° to 200° C. for a time sufficient to drive off the methyl or ethyl alcohol. Thus, in preparing the tetra C<sub>8</sub> to C<sub>16</sub> alkyl ortho silicates, an ester exchange reaction is effected between tetra ethyl ortho silicate and an alcohol selected from the group consisting of octyl, nonyl, decyl, undecyl, dodecyl, tridecyl, tetradecyl, pentadecyl and hexadecyl alcohols.

The organo-silicate condensation products may be obtained as the polymerized hydrolysis products of the esters of ortho silicic acid by controlled hydrolysis of the tetra orthosilicate esters with water. Hydrolysis and condensation or polymerization take place simultaneously with the formation of liquid products which are in general substantially insoluble in hydrocarbon oils and have surface tensions lower than the surface tensions of such oils. Normally mixtures of products in various degrees of polymerization are first obtained. These mixtures after irradiation may be used directly as anti-foam agents. It is generally more advantageous, however, to isolate the higher liquid polymerization products from the total products. In general the effectiveness of the irradiated organo-silicates in preventing foam formation increases with increased molecular weight and boiling point. Also, the higher molecular weight organo-silicates are less soluble in the hydrocarbon oils. Consequently, it is advantageous to irradiate the higher boiling liquid fractions of the products. Separation of the desired fractions may be accomplished by vacuum distillation of the total reaction products.

The irradiated organo-silicates as defined hereinabove are effective foam inhibitors in very low concentration and although they are substantially insoluble in hydrocarbon oils, they are readily dispersible in such oils to form compositions containing stable, fine dispersions of the organo-silicate in hydrocarbon oils, which are substantially resistant to foam formation, without deleteriously modifying the advantageous properties of the oil. Insofar as the organo-silicate condensation products are concerned, the organo-silicate condensation products containing simple organic radicals, such as methyl, ethyl and short-chain alkyl groups are most advantageous inasmuch

as they have exceedingly small solubility in most hydrocarbon oils. For example, an irradiated fraction of the total reaction products obtained on hydrolysis and polymerization of tetramethyl orthosilicate and fractionation at 220° to 240° C. at 0.75 mm., which consists predominantly of a condensation product in which  $n$  is of the order of 3, is markedly effective in concentrations as low as 0.1 percent and less. A similar irradiated fraction obtained by hydrolysis and polymerization of tetraethyl orthosilicate and fractionation of the products to recover the compounds boiling above 290° C. at 1 mm. are also effective in concentrations as low as 0.005 percent and less.

The organo-silicates as defined hereinabove are for all practical purposes substantially oil-insoluble. They are also substantially insoluble in water and aqueous solutions. On the other hand, they can be readily dispersed in hydrocarbon oils to form stable dispersions containing extremely fine particles of irradiated products. In fact, I have prepared oil compositions containing such irradiated organo-silicates dispersed therein, in which a majority of the dispersed particles range from 2.0 to 0.3 micron in diameter or less. Such fine dispersions of these irradiated silicates in oils are very stable and are markedly resistant to foaming. Some oil compositions containing from 5 to 100 parts per million of these compounds finely dispersed therein yield little or no foam when subjected to drastic foaming tests. In fact, some compositions containing as low as 0.05 part per million of a dispersed irradiated silicate show a measurable resistance to foaming. The heavier mineral oils generally require from about 0.00001 to 1 percent by weight to effectively reduce foaming. While the irradiated organo-silicates are for the most part insoluble in mineral oils, some of the organo-silicates may be soluble to a very slight degree. When the irradiated silicate is slightly soluble, the amount of the irradiated silicate used should be sufficiently in excess of its solubility in the oil to give the required amount of dispersed phase necessary to prevent foaming under service conditions. For this reason, the irradiated organo-silicates which are substantially oil-insoluble are most advantageous.

The particle size of the irradiated organo-silicate dispersed in the hydrocarbon oil has a marked effect upon the resistance to foaming so imparted to the oil compositions. In general, oil compositions containing dispersions of the irradiated organo-silicate in which the particles are about 2.0 microns and less in diameter are particularly advantageous for the present purpose. Such oil compositions are very stable in storage and under service conditions, and they have a high resistance to foaming which they retain over long periods of use.

Since good resistance to foaming can be readily obtained with exceedingly small proportions of my new anti-foam agents finely dispersed in the oil, the anti-foam agents of my invention do not deleteriously modify the other properties of such compositions. Accordingly, the desired foam-resisting properties can be imparted to such oils without impairing their effectiveness as lubricants or for other intended uses.

In the commercial practice of this invention, oil compositions may be produced directly in which the anti-foam agent is present in the desired small amount and fine dispersion. However, in certain embodiments of the invention, oil compositions initially containing relatively coarse dispersions and relatively high concentrations of the anti-foam agent may be first prepared and the desired finely dispersed agent concentration may be produced in the oil during use by agitation thereof in the lubricating system, such as by gear pumps and other mechanisms.

Such production of the desired fine dispersions in situ in the oil during use is sometimes advantageous. Of course, the amount of anti-foam agent and the fineness of the dispersion necessary to prevent foaming in a given case vary somewhat with the particular oil and agent employed as well as the service conditions to which the oil composition is subjected.

In preparing my improved oil compositions, the anti-foam agent may be incorporated in the oil or oil composition by any suitable method capable of producing a stable fine dispersion of the agent in the oil. For example, where the anti-foam agent is to be added to a heavy mineral oil, it may first be incorporated in a hydrocarbon oil lighter than the oil to be improved, or other suitable carrier, such as mineral seal oil, gasoline, naphtha, hexane and benzene, and this anti-foam composition may then be introduced into the oil to which it is desired to give anti-foam properties. After such an anti-foam composition has been formed it may be incorporated in the oil or oil composition simply by mixing and agitating the solution therewith. A fine dispersion of the anti-foam agent in the oil is thus obtained. A convenient anti-foam concentrate for such use would contain 1.0 percent of active anti-foam agent. To add 0.001 percent anti-foam agent to the final oil would require the addition of 0.1 percent of the anti-foam concentrate. Where it is desired to form directly a dispersion of the anti-foam agent in the oil, various commercial colloid mills may be employed to disperse finely the agent in the oil. Also, gear pumps may be employed to disperse the anti-foam agent in the oil. The use of such gear pumps is advantageous in many embodiments of this invention, particularly those wherein fine dispersions of the anti-foam agents are produced in situ in the oil. In some instances, the organo-silicate can be added to the oil and then the entire mixture subjected to ionizing radiation. Where such technique is employed, the vehicle should be one that is relatively insensitive to radiation under the conditions employed. Other methods and apparatus may also be employed in dispersing these irradiated agents in oils or oil compositions.

It is sometimes advantageous to first disperse the liquid anti-foam agent in part of the oil and then add this concentrate dispersion to the remainder of the oil. Such concentrate dispersions can be readily prepared as stable uniform compositions. For instance, a mixture of oil and anti-foam agent in the desired proportions may be continuously circulated through a gear pump until a stable concentrate containing a uniform dispersion of the agent is obtained. Thus, standardized concentrates can be prepared which can be added to lubricating compositions as needed. In such case, the desired amount of concentrate is added to the oil composition and the mixture is agitated until uniform.

Also, such concentrates are themselves valuable anti-foam compositions. As they contain a preformed, dispersed, insoluble liquid phase of the desired particle size, they quickly break oil foams, as well as suppress foaming in general. For instance, when added to oil or oil compositions which have foamed, they rapidly destroy the foam present and stop further foaming. In such cases, they can be quickly blended with oils, oil compositions and crude oil and uniformly incorporated therein before serious foaming occurs.

For such purposes, oil concentrates containing from 0.1 to 10 percent by weight and more of finely dispersed anti-foam agent are advantageous. By adding from 0.01 to 10 percent by weight of such concentrates to mineral lubricating oils, improved lubricants having marked resistance to foaming are readily and easily obtained.

The lubricating oils of my invention can contain detergents and/or other "additive" agents including oiliness and extreme pressure agents, such as aromatic chlorine compounds, stabilized chlorinated paraffins, sulfurized fatty oils, and high molecular weight ketones and esters; viscosity index improvers, such as the high molecular

5

and a pour point of 0° F. The tetra(diisobutyl carbonyl)-silicate which was subjected to radiation had a viscosity of 78 SUS at 100° F. and 37.5 SUS at 210° F. The irradiated product as shown hereinabove had no significant change in viscosity and acid value. There was also no noticeable change in color.

Table I

| Composition, percent by weight                                    | A    | B     | C     | D     | E     | F     | G    |
|-------------------------------------------------------------------|------|-------|-------|-------|-------|-------|------|
| Base Oil, 27.9° API—1169 SUS at 100° F.                           | 100  | 99.95 | 99.95 | 99.95 | 99.95 | 99.98 | 99.9 |
| Tetra (diisobutyl carbonyl) silicate, irradiation dosage, mreps.: |      |       |       |       |       |       |      |
| 0                                                                 | 0.05 |       |       |       |       |       |      |
| 6                                                                 |      | 0.05  |       |       |       |       |      |
| 24                                                                |      |       | 0.05  |       |       |       |      |
| 50                                                                |      |       |       | 0.05  |       | 0.02  | 0.1  |
| Foam Test (ASTM D892-46T), Foaming Tendency, ml. at 5 min.:       |      |       |       |       |       |       |      |
| At 75° F.                                                         | 420  | 230   | 170   | 210   | 180   | 120   | 120  |
| At 200° F.                                                        | 130  | 410   | 50    | 50    | 45    | 60    | 45   |

weight polymers of isobutylene and the polymers of methacrylic esters; pour point depressants, such as a condensation product of chlorinated wax and naphthalene and a condensation product of chlorinated wax and phenol followed by further condensation of this reaction product with organic acids; an anti-rust agent such as cocoamine isoamyl octyl orthophosphate; and corrosion and oxidation inhibitors, such as 2,6-di-tertiary butyl-4-methyl phenol, tri-phenyl phosphite, tributyl phosphite, beta naphthol, and phenyl beta naphthylamine. Many of these agents tend to promote foaming. The anti-foam product of my invention, however, can suppress the foaming caused by the addition of such agents to an oil without deleteriously affecting the beneficial characteristics given to the oil by these additives.

The effectiveness of an organo-silicate which has been subjected to ionizing radiation according to my invention in preventing foaming in an oil may be demonstrated by means of ASTM Test Designation D892-46T in which the oil is controllably aerated under fixed conditions so that the results obtained in a series of tests are directly comparable.

The organo-silicate which was subjected to ionizing radiation for purposes of illustrating the invention was tetra(diisobutyl carbonyl) silicate. The tetra(diisobutyl carbonyl) silicate was enclosed in a polyethylene bag and irradiated to various dosages in a Van de Graaff accelerator. The bulk temperature of the tetra(diisobutyl carbonyl) silicate was maintained between about 70° and 200° F. during irradiation. The total energy absorption is shown in connection with the various specific examples.

In preparing samples of oil for the foam test, the agent was added directly to the oil. The mixture thus formed was then blended in a Waring Blender for at least five minutes.

The data summarized in Table I will illustrate the advantageous results obtained by incorporating in a mineral lubricating oil tetra(diisobutyl carbonyl) silicate which had been subjected to irradiation dosages of 6 to 50 megareps. of radiation. A comparison is also made between an oil containing no tetra (diisobutyl carbonyl) silicate and also the same oil containing irradiated and unirradiated tetra(diisobutyl carbonyl) silicate.

The mineral lubricating oil used in preparing the compositions illustrated in Table I was a highly refined paraffinic mineral lubricating oil of SAE 50 grade having an API gravity of 27.9, a viscosity of 1169 SUS at 100° F. and 100 SUS at 210° F., a viscosity index of 101, a flash point (O.C.) of 570° F., a fire point (O.C.) of 625° F.

30

35

40

45

50

55

60

65

70

As shown by the data summarized in Table I, the addition of unirradiated tetra(diisobutyl carbonyl) silicate decreased the amount of foam formed in the oil when tested at 75° F. However, when the same oil was maintained at 200° F., the unirradiated tetra(diisobutyl carbonyl) silicate increased the foaming tendency of the oil. The addition of tetra(diisobutyl carbonyl) silicate which was irradiated to dosages of 6 to 50 megareps. reduced the foaming tendency of the oil at 75° F. and also at 200° F. The improved anti-foam characteristics of compositions of the invention, for example, compositions C to G, is thus readily apparent.

Other specific organo-silicates which when irradiated are useful for the present purpose are tetra methyl ortho silicate condensation products and tetra ethyl ortho silicate condensation products wherein  $n$  in Formula I shown hereinabove is 3. The condensation products of tetra methyl ortho silicate and tetra ethyl ortho silicate can be obtained by heating the respective silicates at refluxing temperature for about 2 to 3 hours in the presence of the corresponding alcohols and water in such proportion as to provide about 0.8 mol of water per mol of silicate. The alcohol and uncondensed ortho silicate are then distilled off at atmospheric pressure. The condensation products are then fractionally distilled at about 1 mm. of mercury pressure. The fractions thus obtained are then subjected to ionizing radiation for a time sufficient for the condensation product to absorb at least 6 megareps. of radiation.

Still other specific organo-silicates include irradiated tetra propyl ortho silicate, tetra butyl ortho silicate, tetra pentyl ortho silicate, tetra hexyl ortho silicate, tetra heptyl ortho silicate, tetra octyl ortho silicate, tetra nonyl ortho silicate, tetra decyl ortho silicate, tetra undecyl ortho silicate, tetra dodecyl ortho silicate, tetra tridecyl ortho silicate, tetra tetradecyl ortho silicate, tetra penta-decyl ortho silicate, tetra hexadecyl ortho silicate, tetra phenyl ortho silicate, tetra tolyl ortho silicate, tetra benzyl ortho silicate, tetra furyl ortho silicate, tetra thiienyl ortho silicate, tetra pyrrol ortho silicate, tetra pyridyl ortho silicate, tetra dichloro phenyl ortho silicate, dimethyl dibutyl ortho silicate, dibutyl diethyl ortho silicate, dimethyl diphenyl ortho silicate, tetra decenyl ortho silicate, tetra butoxyethyl ortho silicate, and their condensation or polymerization products.

The properties of an improved composition of the invention containing 0.05 percent by weight of a 50 mrep. irradiated tetra(diisobutyl carbonyl) silicate are sub-

stantially the same as those of the base oil as shown by the inspection data in the following Table II.

Table II

| Composition                | Mineral Oil | Mineral Oil + 0.05% by weight 50 mrep irradiated tetra(diisobutyl carbonyl) silicate |
|----------------------------|-------------|--------------------------------------------------------------------------------------|
| Gravity, ° API.....        | 27.9        | 27.8                                                                                 |
| Viscosity, SUS:            |             |                                                                                      |
| at 100° F.....             | 1,169       | 1,167                                                                                |
| at 210° F.....             | 100         | 100                                                                                  |
| Viscosity Index.....       | 101         | 102                                                                                  |
| Flash Point (OC), ° F..... | 570         | 565                                                                                  |
| Fire Point (OC), ° F.....  | 625         | 625                                                                                  |
| Pour Point, ° F.....       | 0           | 0                                                                                    |
| Color, ASTM Union.....     | 3-          | 3-                                                                                   |
| Ash, Percent.....          | <0.01       | <0.01                                                                                |

While my invention has been described above with reference to various specific examples and embodiments, it will be understood that the invention is not limited to such illustrative examples and embodiments, and may be variously practiced within the scope of the claims hereinafter made.

I claim:

1. A process of suppressing foaming in a mineral lubricating oil having foaming tendencies comprising dispersing in said oil a small amount, sufficient to improve said foaming tendencies, of a liquid organo-silicate which has been subjected to ionizing radiation for time sufficient for said organo-silicate to absorb about 6 to about 1000 megareps. of radiation while maintaining the bulk temperature of the organo-silicate below its decomposition temperature, said organo-silicate being selected from the group consisting of alkyl, aryl, aralkyl, alkaryl and heterocyclic ortho silicates containing a minimum total of 10 carbon atoms.

2. The process of claim 1 wherein the amount of organo-silicate dispersed in said oil is about 0.00001 to about 1.0 percent by weight of the oil.

3. A process of suppressing foaming in a mineral lubricating oil having foaming tendencies comprising dispersing in said oil a small amount, sufficient to improve said foaming tendencies, of a liquid alkyl ortho silicate which has been subjected to ionizing radiation for a time sufficient for said alkyl ortho silicate to absorb about 6 to about 1000 megareps. of radiation while maintaining the bulk temperature of the alkyl ortho silicate below its decomposition temperature, said alkyl ortho silicate containing a minimum total of 10 carbon atoms.

4. The process of claim 2 wherein the alkyl radical of said alkyl ortho silicate contains from 1 to 16 carbon atoms.

5. A process of suppressing foaming in a mineral lubricating oil having foaming tendencies comprising dispersing in said oil a small amount, sufficient to improve said foaming tendencies, of a liquid tetra alkyl ortho silicate which has been subjected to ionizing radiation for a time sufficient for said tetra alkyl ortho silicate to absorb about 6 to about 1000 megareps. of radiation while maintaining the bulk temperature of the tetra alkyl ortho silicate below its decomposition temperature, said tetra alkyl ortho silicate containing a minimum total of 10 carbon atoms.

6. The process of claim 5 wherein the tetra alkyl ortho silicate is tetra(diisobutyl carbonyl) silicate.

7. A process of suppressing foaming in a mineral lubricating oil having foaming tendencies comprising dispersing in said oil a small amount, sufficient to improve said foaming tendencies, of a liquid ethyl ortho silicate condensation product which has been subjected to ionizing radiation for a time sufficient for said condensation

product to absorb about 6 to about 1000 megareps. of radiation while maintaining the bulk temperature of the condensation product below its decomposition temperature, said condensation product containing a minimum total of 10 carbon atoms.

8. A process of suppressing foaming in a mineral lubricating oil having foaming tendencies comprising dispersing in said oil a small amount, sufficient to improve said foaming tendencies, of a liquid methyl ortho silicate condensation product which has been subjected to ionizing radiation for a time sufficient for said condensation product to absorb about 6 to about 1000 megareps. of radiation while maintaining the bulk temperature of the condensation product below its decomposition temperature, said condensation product containing a minimum total of 10 carbon atoms.

9. A process of suppressing foaming in a mineral lubricating oil having foaming tendencies comprising dispersing in said oil a small amount, sufficient to improve said foaming tendencies, of a liquid organo-silicate which has been subjected to ionizing radiation for a time sufficient for said organo-silicate to absorb about 6 to about 1000 megareps. of radiation while maintaining the bulk temperature of the condensation product below its decomposition temperature, said condensation product containing a minimum total of 10 carbon atoms.

10. A lubricating oil composition of reduced foaming properties comprising a major amount of a mineral lubricating oil having foaming tendencies and a small amount, sufficient to improve said foaming tendencies, of a liquid organo-silicate which has been subjected to ionizing radiation for a time sufficient for said organo-silicate to absorb about 6 to about 1000 megareps. of radiation while maintaining the bulk temperature of the organo-silicate below its decomposition temperature and which is stably dispersed in the oil, said organo-silicate being selected from the group consisting of alkyl, aryl, aralkyl, alkaryl and heterocyclic ortho silicates containing a minimum total of 10 carbon atoms.

11. A lubricating oil composition of reduced foaming properties comprising a major amount of a mineral lubricating oil having foaming tendencies and a small amount,

sufficient to improve said foaming tendencies, of a liquid alkyl ortho silicate which has been subjected to ionizing radiation for a time sufficient for said alkyl ortho silicate to absorb about 6 to about 1000 megareps. of radiation while maintaining the bulk temperature of the alkyl ortho silicate below its decomposition temperature and which is stably dispersed in the oil, said alkyl ortho silicate containing a minimum total of 10 carbon atoms.

12. A lubricating oil composition of reduced foaming properties comprising a major amount of a mineral lubricating oil having foaming tendencies and a small amount, sufficient to improve said foaming tendencies, of a liquid alkyl ortho silicate which has been subjected to ionizing radiation for a time sufficient for said alkyl ortho silicate to absorb about 6 to about 1000 megareps. of radiation while maintaining the bulk temperature of the alkyl ortho silicate below its decomposition temperature and which is stably dispersed in the oil, said alkyl ortho silicate containing a minimum total of 10 carbon atoms.

13. A lubricating oil composition of reduced foaming properties comprising a major amount of a mineral lubricating oil having foaming tendencies and a small amount, sufficient to improve said foaming tendencies, of a liquid tetra alkyl ortho silicate which has been subjected to

ionizing radiation for a time sufficient for said tetra alkyl ortho silicate to absorb about 6 to about 1000 megareps. of radiation while maintaining the bulk temperature of the tetra alkyl ortho silicate below its decomposition temperature and which is stably dispersed in the oil, said tetra alkyl ortho silicate containing a minimum total of 10 carbon atoms.

14. The lubricating oil composition of claim 13 wherein in the tetra alkyl ortho silicate is tetra(diisobutyl carbonyl) silicate.

15. A lubricating oil composition of reduced foaming properties comprising a major amount of a mineral lubricating oil having foaming tendencies and a small amount, sufficient to improve said foaming tendencies, of a liquid ethyl ortho silicate condensation product which has been subjected to ionizing radiation for a time sufficient for said condensation product to absorb about 6 to about 1000 megareps. of radiation while maintaining the bulk temperature of the condensation product below its decomposition temperature and which is stably dispersed in the oil, said condensation product containing a minimum total of 10 carbon atoms.

16. A lubricating oil composition of reduced foaming properties comprising a major amount of a mineral lubricating oil having foaming tendencies and a small amount, sufficient to improve said foaming tendencies, of a liquid methyl ortho silicate condensation product which has been subjected to ionizing radiation for a time sufficient for said condensation product to absorb about 6 to about 1000 megareps. of radiation while maintaining the bulk temperature of the condensation product below its decomposition temperature and which is stably dispersed in the oil, said condensation product containing a minimum total of 10 carbon atoms.

17. A lubricating oil composition of reduced foaming properties comprising a major amount of a mineral lubricating oil having foaming tendencies and about 0.00001 to about 1.0 percent by weight sufficient to improve said foaming tendencies of a liquid organo-silicate which has been subjected to ionizing radiation for a time sufficient for said organo-silicate to absorb about 6 to about 1000 megareps. of radiation while maintaining the bulk temperature of the organo-silicate below its decomposition temperature and which is stably dispersed in the oil, said organo-silicate being selected from the group consisting of alkyl, aryl, aralkyl, alkaryl and heterocyclic ortho silicates containing a minimum total of 10 carbon atoms.

18. A lubricating oil composition of reduced foaming properties comprising a major amount of a mineral lubricating oil having foaming tendencies and about

0.00001 to about 1.0 percent by weight sufficient to improve said foaming tendencies of a liquid tetra alkyl ortho silicate which has been subjected to ionizing radiation for a time sufficient for said tetra alkyl ortho silicate to absorb about 6 to about 1000 megareps. of radiation while maintaining the bulk temperature of the tetra alkyl ortho silicate below its decomposition temperature and which is stably dispersed in the oil, said tetra alkyl ortho silicate containing a minimum total of 10 carbon atoms.

19. The lubricating oil composition of claim 18 wherein in the tetra alkyl ortho silicate is tetra(diisobutyl carbonyl) silicate.

20. A composition adapted to impart foam resisting properties to a mineral lubricating oil having foaming tendencies when added thereto in an amount corresponding to about 0.01 to about 10 percent by weight, comprising a major amount of a hydrocarbon liquid containing from about 0.1 to about 10 percent by weight of a liquid organo-silicate which has been subjected to ionizing radiation for a time sufficient for said organo-silicate to absorb at least about 6 to about 1000 megareps. of radiation while maintaining the bulk temperature of the organo-silicate below its decomposition temperature, said organo-silicate being selected from the group consisting of alkyl, aryl, aralkyl, alkaryl and heterocyclic ortho silicates containing a minimum total of 10 carbon atoms.

21. A lubricating oil composition of reduced foaming properties comprising a major amount of a mineral lubricating oil having foaming tendencies and about 0.00001 to about 1.0 percent by weight, sufficient to improve said foaming tendencies, of tetra(diisobutyl carbonyl) silicate which has been subjected to ionizing radiation for a time sufficient to absorb about 6 to about 50 megareps. of radiation while maintaining the bulk temperature of the tetra(diisobutyl carbonyl) silicate below its decomposition temperature.

#### References Cited in the file of this patent

#### UNITED STATES PATENTS

|    |           |                       |                |
|----|-----------|-----------------------|----------------|
| 40 | 2,375,007 | Larsen et al. -----   | May 1, 1945    |
|    | 2,416,504 | Trautman et al. ----- | Feb. 25, 1947  |
|    | 2,632,736 | Currie -----          | Mar. 24, 1953  |
|    | 2,702,793 | Smith -----           | Feb. 22, 1955  |
|    | 2,766,220 | Kantor -----          | Oct. 9, 1956   |
|    | 2,904,481 | Lawton et al. -----   | Sept. 15, 1959 |

#### OTHER REFERENCES

Charlesby: "Effect of Molecular Weight on the Cross-Linking of Siloxanes by High-energy Radiation," Nature, vol. 173, April 10, 1954, pp. 679,680.

UNITED STATES PATENT OFFICE  
CERTIFICATE OF CORRECTION

Patent No. 3,033,788

May 8, 1962

Charles E. Trautman

It is hereby certified that error appears in the above numbered patent requiring correction and that the said Letters Patent should read as corrected below.

Column 2, line 6, for "he" read -- the --; column 4, line 42, strike out "aralkyl ortho silicates"; column 11, line 54, for the claim reference numeral "2" read -- 3 --.

Signed and sealed this 28th day of August 1962.

(SEAL)

Attest:

ESTON G. JOHNSON

Attesting Officer

DAVID L. LADD  
Commissioner of Patents